

Oct. 14, 1930.

F. A. FAHRENWALD

1,778,213

DIGGING TOOTH WITH HARD METAL CORE

Filed Jan. 21, 1929



Inventor:  
Frank A. Fahrenwald

Witness:  
A. B. Davidson

By Wilkinson, Hurley, Byron & Knight  
Atty's

Patented Oct. 14, 1930

1,778,213

# UNITED STATES PATENT OFFICE

FRANK A. FAHRENWALD, OF CHICAGO, ILLINOIS, ASSIGNOR TO AMERICAN MANGANESE STEEL COMPANY, OF CHICAGO HEIGHTS, ILLINOIS, A CORPORATION OF MAINE

## DIGGING TOOTH WITH HARD-METAL CORE

Application filed January 21, 1929. Serial No. 333,789.

This invention relates to an improved digging tooth having a hard metal core and to a method of producing the improved digging tooth. Digging teeth, such as teeth which are secured to the edge of a dipper, are commonly formed from a manganese steel casting although in some cases dipper teeth have been composed of heat treated alloy steel or even carbon steel but none of these forms have been entirely satisfactory since the edge would not wear away uniformly to maintain a relatively sharp digging edge. It is desired to have the point of the dipper tooth composed of harder metal than the remaining body of the tooth so that the point which receives the greater amount of wear will be worn away at the same rate as the sides of the tooth, that is, the sides will be worn away more rapidly than the harder central point but the contour of the tooth will be maintained and a sharp cutting edge is presented for digging purposes at all times. It has been attempted to use inserts of harder material than the body but these inserts have been cast or forged and held in place only by physical contact with the surrounding metal. In such a construction the insert, which is not homogeneously joined to the body, is liable to break away and other difficulties occur which render such constructions impractical.

It is the purpose of my invention to provide in a dipper tooth or in any article requiring a relatively sharp digging edge, an insert or a plurality of inserts composed of relatively hard and brittle material in a body of relatively soft material which is more tough and ductile and in which the insert is joined to the body by fusion between the surfaces of contact. This may be done by providing an insert of lower melting point than the body and casting the body around the insert whereby the molten body will melt the outer surface of the insert and cause a fusion between the insert and the body.

It is further a purpose of my invention to provide an improved digging tooth having a plurality of inserts of harder material than the body so arranged and spaced that upon wear of the tooth in use the softer body will

be worn away between the inserts and present a serrated digging edge.

A further object of my invention resides in an improved method of forming a dipper tooth having inserts which are harder than the body and in which a body of manganese steel, or other alloy steel, is cast around an insert which, upon heat treatment of the completed article, such as by quenching, will harden the insert to a degree that is harder than the outside body of manganese steel or other alloy steel.

A further object of my invention resides in an improved method of constructing an improved digging tooth in which the inserts of relatively hard material are supported in a mold so that the body of relatively softer material may be poured around the inserts and in which the material composing the body has a higher melting point and will unite with the inserts by fusion.

Further objects and advantages will be more readily apparent as the description proceeds in connection with the attached drawings, in which—

Figure 1 is a side elevation of my improved dipper tooth showing the projecting supporting portion of the inserts which is held in the mold during casting.

Figure 2 is a top plan view of the dipper tooth shown in Figure 1 with the projecting portion of the inserts broken off.

Figure 3 is a sectional elevation on line 3—3 of Figure 1.

Figure 4 is a plan of the lower portion of a mold showing the manner of supporting the inserts therein.

Figure 5 is a plan view of a plurality of inserts secured to a supporting portion.

My invention is disclosed in the drawings in connection with a dipper tooth which is adapted to be secured to the lip or sub-base of an excavating bucket but it will be clearly apparent that a similar construction and method could be followed in connection with other articles having a relatively sharp digging edge.

In the drawings I show a dipper tooth 1 having an acute angle point 2. The tooth is designed with rearwardly extending shanks 100

3 and 4 having a space therebetween but joined by a transverse web 5 in such a manner that the tooth may be joined to an attaching base or directly to the lip of the bucket.

5 Dipper teeth have been commonly composed of alloy steel, generally manganese steel, and it has been necessary to use a steel alloy that is relatively tough and ductile and which will be sufficiently hard so that it will 10 not wear away too rapidly in use, however, even with the use of manganese steel, difficulties are presented in that the point will not maintain its acute angle but will wear away more rapidly at the digging edge and finally 15 assume a blunt point which is not as efficient in digging. It is, therefore, desired to so form the tooth that its contour will be maintained for a substantially long period of time in use.

20 It is my purpose to provide a hard central insert or core or a plurality of such inserts or cores extending inward from the digging edge, thus, I show in Figure 2, which is a plan view of the complete tooth, a plurality 25 of inserts 6. In Figure 3 the inserts are shown in section extending inward substantially the entire length of the tooth body. When the wear reaches the end of the inserts the tooth is discarded.

30 Although I show a plurality of inserts it is my intention to include within my invention a dipper tooth having only one insert. The inserts may be of any suitable cross section such as round, square, rectangular or 35 oblate. The inserts must be of material that is harder than the surrounding body, thus, the outer body may be of low carbon steel which is tough and ductile while the central inserts are composed of high carbon steel 40 which is harder and more brittle. Since the weight of metal comprising the inserts is relatively small as compared with the weight of metal in the dipper tooth, the inserts may be composed of some of the newer alloys 45 which have been found to have high resistance to abrasion but are relatively expensive. It will be noted that the digging edge of the tooth which is composed alternately of the soft body and the hard inserts will wear away 50 more slowly and the relative acute angle contour of the tooth will be substantially maintained. Furthermore, by the use of a plurality of spaced apart inserts, the wear on the tooth will cause the edge to be serrated, 55 thus providing a digging edge which is more effective for digging purposes.

Inserts which have been commonly cast into articles have been joined to the body only by physical contact and are liable to 60 become loose and fall out or break off in use. It is the purpose of my invention to homogeneously join the inserts to the body by fusing the parts at their contacting surfaces. One manner of bringing about the fusion between the inserts and the body consists in

providing a body which is of higher melting point than the inserts and casting the body around the solid inserts whereby the surfaces of the inserts are somewhat dissolved by the molten metal and fusion occurs.

70 One method of casting the tooth will be described in connection with Figures 4 and 5. The member 7 is supported in a recess 8 formed in the bottom part of a mold 9 so that the inserts 6 centrally project into the mold and upon filling the mold with molten steel, the inserts will be surrounded by and fused into the cast body. The steel may be sufficiently over-heated so that it will remain molten in contact with the inserts for 80 a sufficient period to start the dissolving or melting of the surfaces of the inserts and allow fusion to take place.

85 On the article being removed from the mold the projecting portion 7, shown in Figure 1, may be broken off thus leaving the ends of the inserts 6 slightly extending from the digging edge.

90 It will be obvious that my invention may be practiced in many ways and as several instances I may use a metal for the body which is tough and ductile and requires no heat treatment after the casting operation together with an insert of such material that it will be self-hardened and require no further 95 heat treatment. On the other hand, I may use such materials that the inserts will become hard and abrasion resisting and the outer body will become relatively soft, tough and ductile upon heat treatment after the casting is removed from the mold. In the first case I may use a low carbon steel for the body metal and a high carbon steel of lower melting point for the insert material which will not be softened by the casting operation. In the second case I may use manganese steel 100 for the cast body which will become tough and ductile upon quenching and an insert material which will become hard, brittle and abrasion resisting during the quenching 105 operation.

110 Many modifications and changes may be made both in the selection of materials and in the method of forming the article without departing from the spirit of my invention as expressed in the appended claims.

115 I claim:

120 1. An article of manufacture having a digging edge comprising a body of tough, ductile, low carbon steel and a plurality of spaced apart inserts of hard, brittle, high carbon steel extending to the digging edge.

125 2. An article of manufacture having a digging edge comprising a body of tough, ductile, low carbon steel and a plurality of spaced apart inserts of hard, brittle, high carbon steel extending to the digging edge, said body and inserts being united by fusion.

130 3. An article of manufacture having a digging edge comprising a body of manganese

steel and a plurality of spaced apart inserts extending to the digging edge composed of alloy steel which is harder than the manganese steel.

4. An article of manufacture having a digging edge comprising a body of manganese steel and a plurality of spaced apart inserts extending to the digging edge composed of alloy steel which is harder than the manganese steel, said body and inserts being united by fusion.

5. An article of manufacture having a digging edge comprising a cast metal body and a plurality of inserts extending to the digging edge, said inserts being of harder material than the body whereby a serrated digging edge is presented as the edge is worn.

6. An article of manufacture having a digging edge comprising a cast metal body and a plurality of inserts extending to the digging edge, said inserts being of harder material than the body whereby a serrated digging edge is presented as the edge is worn, said inserts being united to the body by fusion.

7. A digging tooth comprising a body and a plurality of spaced apart inserts inwardly extending from the digging edge, said inserts being harder than said body whereby the wear on said tooth will form a serrated edge.

8. A digging tooth comprising a body and a plurality of spaced apart inserts inwardly extending from the digging edge, said inserts being harder than said body whereby the wear on said tooth will form a serrated edge, said body and inserts being united by fusion.

Signed at Chicago, Illinois, this 16th day of January, 1929.

FRANK A. FAHRENWALD.

40

45

50

55

60

65